# EUROPEAN PATENT SPECIFICATION

(11) **EP 3 486 034 B1**
(45) Date of publication and mention of the grant of the patent: **22.06.2022**
(21) Application number: 17856053.8
(22) Date of filing: 25.09.2017
(51) Int. Cl.: B24C 1/04, B24C 5/04

(54) **A DRILLING METHOD OF FORMING A HOLE HAVING A DESIRED DIAMETER IN A FIBER REINFORCED PLASTIC WORKPIECE**
EIN BOHRVERFAHREN ZUR HERSTELLUNG EINES LOCHES MIT EINEM GEWÜNSCHTEN DURCHMESSER IN EINEM WERKSTÜCK AUS FASERVERSTÄRKTEM KUNSTSTOFF
UN PROCÉDÉ DE PERÇAGE POUR FORMER UN TROU AYANT UN DIAMÈTRE SOUHAITÉ DANS UNE PIÈCE EN PLASTIQUE RENFORCÉE DE FIBRES

(30) Priority: 28.09.2016 JP 2016189185; 08.03.2017 JP 2017043513
(43) Date of publication of application: 22.05.2019
(73) Proprietor: Sintokogio, Ltd., Nagoya-shi, Aichi 450-6424 (JP)
(72) Inventor: INOUE Kouichi, Kitanagoya-shi Aichi 481-8678 (JP)
(74) Representative: Hoffmann Eitle
(86) International application number: PCT/JP2017/034538
(87) International publication number: WO 2018/062101

(56) References cited:
- WO-A1-2007/091476
- WO-A1-2014/089224
- CN-A- 105 304 576
- JP-A- H0 469 167
- JP-A- S58 175 632
- JP-A- 2002 353 425
- JP-A- 2002 353 425
- JP-A- 2012 196 751
- JP-A- 2013 146 851
- US-A- 4 612 737
- US-A1- 2002 071 983

## Description

### Technical Field

The present disclosure relates to a drilling method of forming a hole having a desired diameter in a fiber reinforced plastic workpiece comprising steps of:
- disposing a resist layer; and
- ejecting blasting abrasives to the workpiece through the resist layer to cut a portion, which is exposed from the opening, in the workpiece.

### Background Art

A fiber-reinforced plastic (FRP) is a composite material in which reinforcing fiber (glass fiber, carbon fiber, aramid fiber, polyethylene fiber, cylon fiber, boron fiber, and the like) is put into a resin (a polyester resin, a vinyl ester resin, an epoxy resin, a phenol resin, and a thermoplastic resin) to improve strength. The FRP has been used in a wide range of fields such as daily necessities, sporting goods, automobiles, and aerospace applications.

The FRP may be subjected to drilling to improve joining and sound absorbency in some cases. As a method of forming a hole in an FRP workpiece, drilling performed by using a drill, and sandblasting are used. For example, US 4,612,737 A and JP 2012-196751 A disclose a configuration in which a resist layer having sandblast resistance is disposed on a surface of the workpiece, and a region which is not covered with the resist layer in the workpiece is removed by sandblasting.

### Citation List

### Patent Literature

US 4,612,737 A relates to grit blast drilling of advanced composite perforated sheet. Described is a method and resulting product produced by attaching a prepared maskant of a desired perforation pattern to cured compound contoured or flat advanced composite materials, directing a narrow stream of highly abrasive grit material of a selected particle size range through a relatively large nozzle under selected high pressure toward the maskant perforations at a very small angle relative to the perforation walls until perforations are formed in the advanced composite material according to the stencil perforation pattern.

JP 2002-353425 A describes a saphire substrate and manufacturing method therefor. Provided is a method, except for wet etching, as a method for forming a through-hole in the manufacturing method of a substrate which is constituted of saphire and which has a through-hole whose diameter is under 0.1 mm. In the method, the saphire substrate is masked, and the through-hole is formed by blast working method.

JP 2012-196751 A relates to a method of boring fiber-reinforced plastic and a fiber-reinforced plastic finished product. In this method of boring a fiber-reinforced plastic, a resist layer having sand blast resistance is fitted closely to a fiber-reinforced plastic, and after the fiber-reinforced plastic is removed by sand blasting from the portion with no resist layer, the resist layer is peeled and removed.

US 2002/071983 A relates to flow field plates and the manufacture thereof, for use in fuel cells. The method of manufacture comprises particulate etching of a plate material using a particulate etchant (e.g. sand blasting), a particulate etchant accelerator and a particulate etchant-resistant patterned mask, such that a fluid flow pattern determined by the pattern design on said mask is formed on the plate material.

### Summary of Invention

### Technical Problem

In drilling performed by using a drill, in a case where the number of holes to be processed is large, a processing time is lengthened, and thus the drilling is not preferable from the viewpoint of productivity. In addition, in the drilling performed by using a drill, fluffing may occur in the vicinity of a hole formed in a workpiece, or peeling-off may occur on a surface of the workpiece.

In addition, as in a method described in US 4,612,737 A , even in a case where a hole is formed in a workpiece by sandblasting, fluffing or peeling-off may occur in the workpiece although the degree of occurrence is lower in comparison to the drilling performed by using a drill.

Accordingly, it is desired to form a hole in the fiber-reinforced plastic while suppressing occurrence of fluffing and peeling-off.

### Solution to Problem

According to the present invention, there is provided a drilling method of forming a hole having a desired diameter in a fiber-reinforced plastic workpiece, as defined in claim 1. The method includes disposing a resist layer, in which an opening having a diameter smaller than the desired diameter is formed, on the workpiece and ejecting blasting abrasives to the workpiece through the resist layer to cut a portion, which is exposed from the opening, in the workpiece while cutting a peripheral edge portion of the opening of the resist layer.

When the blasting abrasives are continuously projected to the workpiece through the resist layer, the blasting abrasives passing through the opening of the resist layer enters a downward side of the resist layer, and thus peeling-off may occur on a surface of the workpiece. When the peeling-off occurs, reinforcing fibers of the workpiece are exposed on the surface of the workpiece as fluffing. In the method according to the aspect, the blasting abrasives are ejected to the workpiece through the resist layer in which the opening having the diameter smaller than the desired diameter is formed. In this method, the blasting abrasives collide with the resist layer and cuts a peripheral edge portion of the opening formed in the resist layer, the diameter of the opening is gradually enlarged with the passage of a processing time. In this manner, when the hole is formed in the workpiece while gradually enlarging the diameter of the opening in the resist layer, even when peeling-off occurs in the workpiece, a peeled-off portion is removed along the progress of processing of the workpiece. As a result, it is possible to suppress occurrence of peeling-off and fluffing on the surface of the workpiece after processing.

Further, in the inventive drilling method according to claim 1, a ratio of the diameter of the opening to the desired diameter is 0.84 or more and 0.94 or less. When the ratio of the diameter of the opening to the desired diameter is set as described above, it is possible to efficiently perform processing while maintaining accuracy in a hole diameter after processing.

In one embodiment, in the step of ejecting the blasting abrasives to the workpiece, the blasting abrasives may be ejected toward the workpiece from a nozzle, and an angle formed by a surface of the workpiece and a ejecting direction of the blasting abrasives from the nozzle may be 90° ± 5°. When the blasting abrasives are ejected to the workpiece at this angle, it is possible to suppress occurrence of peeling-off on the surface layer of the resin. As a result, it is possible to suppress fluffing.

In one embodiment, the nozzle may be configured to suck the blasting abrasives by introducing compressed air to the inside of the nozzle to eject the blasting abrasives with the compressed air as a solid-gas two-phase flow. The fiber-reinforced plastic is a difficult-to-cut material with respect to blast processing, and thus a considerable time is necessary until processing is completed. In this embodiment, the blasting abrasives can be continuously ejected from the nozzle, it is possible to improve processing efficiency.

In one embodiment, the workpiece may comprise the fiber-reinforced plastic in which a cut reinforcing fibers are dispersed in a resin. In this type of fiber-reinforced plastic, the reinforcing fibers are dispersed without directionality. Accordingly, in a conventional drilling method, a surface may be peeled off from the reinforcing fibers as the origin, and the fiber-reinforce plastic may be broken. In contrast, according to the drilling method of the one embodiment, even in the workpiece as described above, it is possible to suppress occurrence of peeling-off or fluffing on the surface of the workpiece.

In one embodiment, the workpiece may comprise the fiber-reinforced plastic in which woven reinforcing fibers infiltrate into a resin. In this type of fiber-reinforced plastic is obtained by alternately laminating reinforcing fibers that are woven in a cloth shape and a resin. Accordingly, in the conventional drilling method, inter-layer peeling-off may occur, and the fiber-reinforced plastic may be broken. According to the drilling method of the one embodiment, even in the workpiece as described above, it is possible to suppress occurrence of peeling-off or fluffing on the surface of the workpiece.

In one embodiment, the resist layer may be a polymer including unsaturated polyurethane or an abrasion-resistant rubber as a main component. In a case of using the polymer as a material of the resist layer, when drilling the workpiece, the resist layer is suppressed from being excessively deformed, and thus it is possible to enhance dimensional accuracy of a hole that is formed in the workpiece.

In one embodiment, the fiber-reinforced plastic may have a plate shape having a thickness of 1.0 mm or more and 2.0 mm or less, and an angle formed by a plane perpendicular to a central axis line of the hole and a wall surface defining the hole may be 80° or more and 90° or less. When the angle formed by the plane perpendicular to the central axis line of the hole and the wall surface defining the hole is an angle of 80° or more and 90° or less, it is possible to improve uniformity of a hole diameter in a thickness direction of the fiber-reinforced plastic.

Furthermore, the plate shape stated here includes not only a flat plate shape but also a curved plate shape.

### Advantageous Effects of Invention

According to the aspect and embodiments of the present disclosure, it is possible to form a hole in a fiber-reinforced plastic while suppressing occurrence of fluffing and peeling-off.

### Brief Description of Drawings

FIG. 1 is a front view illustrating a sandblast machine that is used in one embodiment in a partially cut-out manner.
FIG. 2 is a flowchart illustrating a drilling method of one embodiment.
FIG. 3 is a view schematically illustrating a scanning trajectory of a workpiece of one embodiment.
FIG. 4 is a cross-sectional view illustrating a workpiece to which a drilling method of one embodiment is applied.
FIG. 5 is a cross-sectional view illustrating a workpiece to which a conventional drilling method is applied.

### Description of Embodiments

Hereinafter, various embodiments will be described in detail with reference to the accompanying drawings. Furthermore, the same reference sign will be given to the same or equivalent portion in the drawings, and redundant description for the same or equivalent portion will be omitted. In addition, it is not necessary for dimension ratios of the drawings to match actual dimension ratios. Furthermore, right and left directions and upper and lower directions in description represent directions in the drawings unless otherwise stated.

FIG. 1 is a front view illustrating a sandblast machine 01 according to one embodiment in a partially cut-out manner. The sandblast machine 01 is a device that projects blasting abrasives to a fiber-reinforced plastic workpiece W (workpiece) and forms a hole in the workpiece W. As illustrated in FIG. 1, the sandblast machine 01 includes a housing 10, a fixed-quantity supply mechanism 20, a separation mechanism 30, a suction mechanism 40, a nozzle 50, and a control device 60.

The housing 10 constitutes a processing chamber R on an inner side thereof. A door 11 is provided in a front surface of the housing 10, and an operator can access the processing chamber R by opening the door 11. A nozzle fixture 12, a processing table 13, and a movement mechanism 14 are provided in the processing chamber R.

The nozzle fixture 12 is a mechanism that holds the nozzle 50, and can move the nozzle 50 along a height direction. Accordingly, the nozzle fixture 12 is configured to freely adjust a distance between the nozzle 50 and the workpiece W.

The movement mechanism 14 is provided on a frame 15 that is provided on a lower side of the housing 10, and is disposed on a downward side of the nozzle 50. In one embodiment, the movement mechanism 14 may be plate-shaped body in which a plurality of through-holes are formed. When the through-holes are formed in the movement mechanism 14, it is possible to allow blasting abrasives, which is ejected from the nozzle 50, to propagate toward the bottom of the housing 10.

The processing table 13 is provided on the movement mechanism 14 and supports the workpiece W that is placed on the processing table 13. For example, the movement mechanism 14 is configured to convey the processing table 13 and the workpiece W supported on the processing table 13 in a horizontal direction by a driving force of a motor. For example, the movement mechanism 14 is an X-Y stage that extends in the horizontal direction and moves the workpiece W in an X direction and a Y direction which are perpendicular to each other (refer to FIG. 3).

The fixed-quantity supply mechanism 20 is provided on an upper side of the processing chamber R. The fixed-quantity supply mechanism 20 includes a storage hopper 21 and a conveyance path 22, and supplies blasting abrasives in the storage hopper 21 to the nozzle 50 in a fixed quantity through the conveyance path 22. Furthermore, a structure of the fixed-quantity supply mechanism 20 is not limited as long as the fixed-quantity supply mechanism 20 can supply a constant amount of blasting abrasives to the nozzle 50. For example, as the fixed-quantity supply mechanism 20, a screw feeder, a vibration feeder, and a table feeder can be used. In the embodiment illustrated in FIG. 1, the screw feeder is used as the fixed-quantity supply mechanism 20.

The separation mechanism 30 is provided on an upper side of the storage hopper 21 of the fixed-quantity supply mechanism 20. The separation mechanism 30 is connected to the storage hopper 21 of the fixed-quantity supply mechanism 20. The separation mechanism 30 has an approximately inverted pyramid shape, collects used blasting abrasives, and classifies the blasting abrasives into a blasting abrasives that can be reused, and dust. One end of a first transport pipe P1 is connected to the separation mechanism 30. The other end of the first transport pipe PI is connected to the bottom of the housing 10. Accordingly, a space in the processing chamber R and a space in the fixed-quantity supply mechanism 20 communicate with each other through the first transport pipe PI. In the embodiment illustrated in FIG. 1, a cyclone type classifier is used as the separation mechanism 30. However, as the separation mechanism 30, arbitrary classifiers such as a wind power type classifier, a screen type classifier can be used.

In addition, one end of a second transport pipe P2 is connected to the separation mechanism 30. The other end of the second transport pipe P2 is connected to the suction mechanism 40. The suction mechanism 40 is a mechanism that sets the processing chamber R to negative pressure in order for the blasting abrasives not to be leaked to the outside of the processing chamber R, and suctions particles including the blasting abrasives that are ejected. The suction mechanism 40 collects light particles (a blasting abrasives that becomes a size that is not appropriate for reuse, and chip powders of the workpiece W and a sheet 70) which are classified in the separation mechanism 30 (cyclone type classifier) through the second transport pipe P2. In addition, the suction mechanism 40 has a function of setting an internal space of the separation mechanism 30 to negative pressure, and transporting the blasting abrasives, which is used and collected at the bottom of the housing 10, to the separation mechanism 30.

The nozzle 50 is a mechanism that ejects the blasting abrasives to the workpiece W, and includes a nozzle holder 51, an air nozzle 52, and an ejecting nozzle 53. The nozzle holder 51 is connected to the fixed-quantity supply mechanism 20 through a blasting abrasive hose H2. A compressor C is connected to the air nozzle 52 through an air hose HI. In one embodiment, an electromagnetic valve VL1 and a valve VL2 may be provided between the air nozzle 52 and the compressor C. When the compressor C is operated, compressed air is ejected from the air nozzle 52, and the inside of the nozzle holder 51 becomes negative pressure. According to this, the blasting abrasives stored in the storage hopper 21 is suctioned into the nozzle holder 51 through the conveyance path 22 and the blasting abrasive hose H2, is mixed with the compressed air in the nozzle holder 51, and is ejected as a solid-gas two-phase flow from an ejecting port of the ejecting nozzle 53 toward the workpiece W. The nozzle 50 having the above-described configuration can continuously eject the blasting abrasives, and thus it is possible to continuously process the workpiece W over a long time.

Furthermore, a so-called direct pressure type nozzle can be used as a nozzle of another type. The direct pressure type nozzle has more excellent cutting capacity in comparison to the nozzle 50 of this embodiment, but it is difficult to continuously perform processing over a long time.

Examples of a blasting abrasives that is ejected from a nozzle include a metal or nonmetal shot, grid, or cut-wire, ceramic-based particles (alumina-based particles, silicon carbide-based particles, zircon-based particles, and the like), natural stone particles (emery, silica stone, diamond, and the like), plant-based particles (a shell of a walnut, a peach stone, an apricot stone, and the like), resin-based particles (nylon, melamine, urea, and the like), and the like. The fiber-reinforce plastic is a difficult-to-cut material. Accordingly, when selecting a relatively hard material as the blasting abrasives, it is possible to efficiently cut the workpiece W.

The control device 60 is a computer including a processor, a storage unit, an input device, a display device, and the like, and controls respective units of the sandblast machine 01. In one embodiment, the control device 60 transmits a control signal to the movement mechanism 14, the fixed-quantity supply mechanism 20, the suction mechanism 40, and the electromagnetic valve VL1, and controls positions of the movement mechanism 14 in the X direction and the Y direction, an operation of the fixed-quantity supply mechanism 20, an operation of the suction mechanism 40, and opening and closing of the electromagnetic valve VL1, and the like. As a control device, various operation devices such as a personal computer, a motion controller such as a programmable logic controller (PLC) and a digital signal processor (DSP), a high-function portable terminal, a high-function portable telephone, and the like can be used.

Hereinafter, description will be given of a drilling method by the sandblast machine 01 of one embodiment with reference to FIG. 2. In this method, a hole H having a desired diameter d₁ is formed in the fiber-reinforced plastic workpiece W. The workpiece W has a flat plate shape, and includes an upper surface (front surface) 82 and a lower surface (rear surface) 84 opposite to each other (refer to FIG. 4). The hole H to be formed in the workpiece W is a through-hole that extends from the upper surface 82 to the lower surface 84, and is opened to the upper surface 82 and the lower surface 84. In the hole H, an opening (first opening) 86 on the upper surface 82 side has the desired diameter d₁. In other words, the hole H to be formed in the workpiece W is a through-hole including the opening 86 having an area (first area) corresponding to the desired diameter d₁ on the upper surface 82 side. Hereinafter, description will be given of an example in which the workpiece W is constituted by a glass fiber-reinforced plastic (GFRP) that is one kind of the fiber-reinforced plastic.

Furthermore, the desired diameter d₁ of the opening 86 represents a length of the widest portion in the diameter of the opening 86. For example, in a case where the opening 86 has an elliptical shape, the major axis of the ellipse becomes the desired diameter d₁. In a case where the opening 86 has a polygonal shape, a length of the longest straight line among straight lines which connect arbitrary two corners of the polygon becomes the desired diameter d₁. Hereinafter, description will be given of an embodiment in which the opening 86 has a circular shape. In this embodiment, the diameter of the opening 86 becomes the desired diameter d₁.

### <S1: Preparation of Resist Layer>

In a drilling method according to one embodiment, first, a step S1 is performed. In the step S1, a sheet 70 that functions as a resist layer is prepared. The sheet 70 is constituted by a material that is softer than the blasting abrasives and is capable of absorbing an impact force of the blasting abrasives. Accordingly, the sheet 70 has blast resistance that is higher than that of the workpiece W constituted by the fiber-reinforced plastic.

One or a plurality of openings (second openings) 71 are formed in the sheet 70 (refer to FIG. 4). Each of the openings 71 has a shape corresponding to a shape of the opening 86 of the hole H. For example, the opening 71 has a planar shape such as a circular shape, an elliptical shape, and a polygonal shape in correspondence with the shape of the opening 86. In one embodiment, the opening 71 of the sheet 70 has the same shape as that of the opening 86 of the workpiece W. However, a diameter d₂ of the opening 71 is set to smaller than the desired diameter d₁. In other words, the opening 71 has an area (second area) that is smaller than the area of the opening 86. A ratio (d₂/d₁) of the diameter d₂ of the opening 71 to the desired diameter d₁ may be set in a range of 0.84 to 0.94, particularly, in a range of 0.90 to 0.94. As to be described later, when the ratio is excessively small, a collision chance between the workpiece W and the blasting abrasives are excessively less, and thus a drilling time is lengthened. In contrast, the ratio is excessively large, peeling-off is likely to occur in a surface layer of the workpiece W. Here, the diameter d₂ of the opening 71 represents the largest diameter among diameters defined by the opening 71. For example, in a case where the planar shape of the opening 71 is set to an elliptical shape, the major axis of the opening 71 of the elliptical shape becomes the diameter d₂. In a case where the planar shape of the opening 71 is set to a polygonal shape, a length of the longest straight line among straight lines which connect arbitrary two corners of the polygon becomes the diameter d₂. Hereinafter, description will be given of an embodiment in which the planar shape of the opening 71 is a circular shape. In this embodiment, the diameter of the opening 71 becomes the diameter d₂.

As a material of the sheet 70, for example, thermoplastic resins such as various rubbers, nylon, polyethylene (PE), polypropylene (PP), polyurethane, and acrylic can be used. For example, as the material of the sheet 70, an abrasion-resistant rubber can be used. Abrasion resistance of a rubber can be easily adjusted by changing a blending ratio of a filling reinforcing material such as calcium carbonate to a natural rubber or a synthetic rubber that is a main raw material. Accordingly, when using the abrasion-resistant rubber as the material of the sheet 70, it is possible to easily obtain a resist material having abrasion resistance that is appropriate for drilling. In one embodiment, an abrasion-resistance rubber in which a reinforcing filling material is blended to a natural rubber or a synthetic rubber in a ratio of 60 wt% to 70 wt% can be used as the material of the sheet 70.

In addition, polyurethane is comprehensively excellent in elasticity, a thermal deformation temperature, and impact strength. Accordingly, when using polyurethane as the material of the sheet 70, it is possible to improve accuracy of a diameter of the hole H that is formed in the workpiece W. In addition, it is possible to easily form the opening 71 having a small diameter (for example, φ 2 mm or less) in the polyurethane sheet 70. As to be described later, in a method of one embodiment, a portion exposed from the opening 71 in the workpiece W is cut while cutting a peripheral edge portion 72 of the opening 71 in the sheet 70 by blasting abrasives. At this time, when the peripheral edge portion 72 of the sheet 70 is cut more than necessary, fluffing or peeling-off may occur on a surface of the workpiece W or dimensional accuracy may deteriorate due to the cutting. Accordingly, the material of the sheet 70 is selected in consideration of elasticity, a thermal deformation temperature, and impact force resistance. For example, unsaturated polyurethane is comprehensively excellent in elasticity, a thermal deformation temperature, and Charpy impact strength, and thus the sheet 70 may be constituted by a polymer that includes unsaturated polyurethane as a main component. In addition, a content rate of the unsaturated polyurethane may be set to 50 wt% or more, or 50 wt% to 70 wt%.

In one embodiment, the sheet 70 may be formed from a photosensitive resin that is shaped in a film shape. When forming the sheet 70 from the photosensitive resin, first, a transparent pattern mask in which an opening pattern is printed is disposed on the sheet 70, the sheet 70 is irradiated with ultraviolet rays from an ultraviolet ray emission source provided on an upper side of the sheet 70 through the pattern mask. In the sheet 70, a region that does not overlap a printed pattern is cured through irradiation of ultraviolet rays. However, a portion that overlaps the printed opening pattern become shadow, and is not cured. Subsequently, the sheet 70 after being irradiated with ultraviolet rays is washed out by using a development solution, and thus the uncured region of the sheet 70 is removed. A plurality of the openings 71 can be formed in the sheet 70 through a series of processes as described above.

In addition, in the step S1, the prepared sheet 70 is disposed on the workpiece W. In one embodiment, the sheet 70 may have stickiness. In this case, after the sheet 70 is stuck to an upper surface of the workpiece W, pressure is reduced in a vacuum chamber. According to this, it is possible to closely stick the sheet 70 onto the workpiece W. In addition, when the workpiece W is subsequently heated at a temperature of 60°C to 90°C, the workpiece W and the sheet 70 can be firmly and closely stuck to each other.

### <S2: Preparation of Sandblast Machine>

Subsequently, in a drilling method according to one embodiment, a step S2 is performed. In the step S2, the sandblast machine 01 is prepared. In the step S2, first, the suction mechanism 40 is operated for suctioning of the processing chamber R. Subsequently, locking of the door 11 is released to open the door 11, and a predetermined amount of blasting abrasives are put into the processing chamber R by an operator as an example. Subsequently, the blasting abrasives are transported to the storage hopper 21 of the fixed-quantity supply mechanism 20 through the first transport pipe PI and the separation mechanism 30 due to a suction force of the suction mechanism 40. Then, the door 11 is closed and locked. The processing chamber R becomes negative pressure due to suctioning of the suction mechanism 40, and thus external air flows into the processing chamber R from a suction hole (not illustrated) provided to communicate with the outside.

In the step S2, for example, the control device 60 of the sandblast machine 01 is operated to set the electromagnetic valve VL1, which is provided in a path through which compressed air is supplied to the nozzle 50, to "open", and to set the fixed-quantity supply mechanism 20 to "ON". Through the setting, the blasting abrasives are supplied to the nozzle 50, and are ejected from the nozzle 50. When the blasting abrasives are ejected from the nozzle 50, the degree of opening of the valve VL2 that adjusts compressed air supply pressure is adjusted, and thus a ejected velocity of the blasting abrasives are adjusted.

Subsequently, the control device 60 of the sandblast machine 01 is operated to set the electromagnetic valve VL1 to "close", and to set the fixed-quantity supply mechanism 20 to "OFF". Through the setting, ejecting of the blasting abrasives from the nozzle 50 are stopped. Then, the door 11 is opened, and the workpiece W is placed on the processing table 13 and is fixed thereto. Subsequently, the nozzle fixture 12 is operated to adjust a distance and an angle between the nozzle 50 and the workpiece W. When the above-described processes are finished, the door 11 is closed and locked. Furthermore, the workpiece W that is placed on the processing table 13 may be a plate-shaped body having a thickness of 1.0 or more and 2.0 mm or less.

Subsequently, in the step S2, processing conditions such as a movement trajectory (distances in the X direction and the Y direction in FIG. 3) and a movement velocity of the movement mechanism 14, and the number of times of scanning are input to the control device 60.

### <S3: Drilling Process>

Subsequently, a step S3 is performed. In the step S3, as to be described later, the blasting abrasives are ejected toward the workpiece W through the sheet 70 to cut a portion exposed from the opening 71 in the workpiece W while cutting the peripheral edge portion 72 of the opening 71 in the sheet 70. Hereinafter, an example of the step S3 will be described in detail.

In the step S3, first, the control device 60 is operated to set the electromagnetic valve VL1 to "open" and to set the fixed-quantity supply mechanism 20 to "ON". According to this, the blasting abrasives are ejected from the nozzle 50. Subsequently, the movement mechanism 14 is set to "ON", and the movement mechanism 14 operates so that the workpiece W is moved in a horizontal direction. For example, as illustrated in FIG. 3, the movement mechanism 14 repeats movement of the workpiece W in a +X direction by a predetermined distance, and movement of the workpiece W in a -X direction after deviating a position of the workpiece W in a +Y direction by a predetermined pitch. According to this, the workpiece W is scanned in a comb-tooth shape with respect to an ejecting region A of the blasting abrasives. The movement mechanism 14 moves the workpiece W along a scanning trajectory T to allow the blasting abrasives to collide with the entire surface of the workpiece W in an approximately uniform manner. In one embodiment, the scanning is performed in a plurality of times to form the hole H in the workpiece W. An ejecting port of the nozzle 50 may have rectangular planar shape. When the ejecting port of the nozzle 50 has a rectangular planar shape and is disposed in such a manner that a long side of the ejecting port matches the Y direction, it is possible to enlarge a collision area of the blasting abrasives when the workpiece W is scanned in the X direction. As a result, it is possible to improve processing efficiency of the workpiece W.

As described above, when the workpiece W is conveyed in the X direction and the Y direction by the movement mechanism 14, in the workpiece W, the hole H is formed in a region that is not covered with the opening 71 of the sheet 70. Here, as illustrated in FIG. 4, the blasting abrasives are projected from the nozzle 50 toward a region that includes the opening 71 and the peripheral edge portion 72 of the opening 71. Accordingly, in the step S3, as illustrated in FIG. 4, a region exposed from the opening 71 in the workpiece W is cut while the peripheral edge portion 72 of the opening 71 is cut. The sheet 70 has blast resistance higher than that of the fiber-reinforced plastic that constitutes the workpiece W, and thus the peripheral edge portion 72 of the sheet 70 is cut slowly in comparison to the workpiece W. Accordingly, in the step S3, the region exposed from the opening 71 in the workpiece W is cut in such a manner that a cut area of the workpiece W does not become excessive while gradually enlarging a diameter (area) of the opening 71 of the sheet 70. As a result, the peeling-off of the workpiece W in a surface layer is suppressed. In the step S3, projection of the blasting abrasives continues until the diameter of the hole H formed in the workpiece W becomes the desired diameter d₁.

FIG. 5 illustrates a shape of the hole H that is formed in the workpiece W when the diameter d₂ of the opening 71 and the desired diameter d₁ are set to be the same as each other. That is, FIG. 5 illustrates a conventional method in which the hole H having the desired diameter d₁ is directly formed in the workpiece W without cutting the peripheral edge portion 72 of the sheet 70. In a case where the fiber-reinforced plastic that constitutes the workpiece W has a structure in which a cut reinforcing fibers are dispersed in a resin, when the blasting abrasives are projected to the workpiece W, the reinforcing fibers dispersed without directionality becomes the origin of fracture, and thus peeling-off occurs on a surface of the workpiece W. In addition, in a case where the fiber-reinforce plastic that constitutes the workpiece W has a structure in which a woven reinforcing fibers infiltrate into a resin, the reinforcing fibers having a cloth shape becomes the origin of fracture, and thus peeling-off occurs on a surface of the workpiece W. When cutting further continues after the peeling-off occurs, the diameter of the hole H formed in the workpiece W finally becomes larger than the desired diameter d₁, and a surface layer portion does not become a circle shape. In addition, fluffing of the reinforcing fibers occur on a wall surface of the hole H (refer to a portion surrounded by a circle in the same drawing).

In the case where an ejection flow of the blasting abrasives are captured microscopically, when the ejection flow flows along the surface of the workpiece W, the surface layer of the workpiece W is likely to be peeled off due to the characteristics of the fiber-reinforced plastic. When peeling-off occurs in the surface layer of the workpiece W, the reinforcing fibers are exposed to surface layer, and thus fluffing occurs. Furthermore, the ejection flow flows in a direction conforming to a wall surface of the opening of the sheet 70 (that is, a direction perpendicular to the X direction and the Y direction), it is possible to suppress peeling-off on the surface layer of the workpiece W. As a result, it is possible to suppress fluffing of the reinforcing fibers. In a case where the fiber-reinforced plastic that constitutes the workpiece W has a structure in which woven reinforcing fibers infiltrate into a resin, the blasting abrasives collide with the workpiece W in a direction in which the reinforcing fibers of the workpiece W is cut, and thus it is possible to further suppress fluffing of the reinforcing fibers. In addition, in a case where the ejection flow is greatly inclined to the surface of the workpiece W, collision energy of the blasting abrasives are not sufficient. Accordingly, the hole H may not be formed in the workpiece W, the reinforcing fibers may not be cut, or the reinforcing fibers may be exposed on an outer peripheral surface of the hole H as fluffing. Here, in one embodiment, the nozzle 50 may be disposed at an angle of 85° to 95° (that is, in a range of 90° ± 5°) with respect to the surface of the workpiece W. In other words, the nozzle 50 is disposed so that an angle made by the surface of the workpiece W and an ejecting direction of the blasting abrasives becomes 85° or more and 95° or less.

When processing is performed so that an angle of a wall surface of the hole H formed in the workpiece W becomes appropriate, the processing is advantageous in performance. For example, the hole H formed in the workpiece W is provided for joining, the higher the perpendicularity of a wall surface defining the hole H is, the more a clearance between a joining member such as a bolt and the wall surface of the hole H becomes uniform in a thickness direction. As a result, it is possible to suppress backlash after joining. In addition, in a case where the hole H formed in the workpiece W is provided to improve sound absorbency, the higher the perpendicularity of the wall surface defining the hole H is, the further sound reflection due to the wall surface of the hole H is prevented. As in the examples, it is preferable that the angle of the wall surface with respect to a plane perpendicular to a central axis line AX of the hole H is close to 90° from the viewpoint of performance. However, as it is close to 90°, productivity further deteriorates. Accordingly, the angle of the wall surface that constitutes the hole H with respect to the plane perpendicular to the central axis line AX of the hole H may be 80° to 90°, or 80° to 85° from the viewpoints of productivity and performance.

Particles including the blasting abrasives projected to the workpiece W in the step S3 are collected at the bottom of the housing 10, and is transported to the separation mechanism 30 through the first transport pipe PI due to a suction force of the suction mechanism 40. The particles transported to the separation mechanism 30 are separated into a blasting abrasives that can be reused and dust in the separation mechanism 30. The blasting abrasives that can be reused are accumulated in the storage hopper 21, and light dust is suctioned to the suction mechanism 40 and is collected by a collection filter provided inside the suction mechanism 40. The blasting abrasives that are accumulated in the storage hopper 21 and can be reused are transported to the nozzle 50 in a constant amount, and are ejected again toward the workpiece W.

### <S4: Recovery Process>

After forming the hole H in the workpiece W in the step S3, a step S4 is performed. In the step S4, the control device 60 is operated to set the movement mechanism 14 to "OFF", to set the electromagnetic valve VL1 to "close", and to set the fixed-quantity supply mechanism 20 to "OFF", respectively. Then, locking of the door 11 is released to open the door 11, and the workpiece W is recovered from the processing chamber R. Subsequently, after the sheet 70 stuck to the workpiece W is peeled off, the blasting abrasives and dust which adhere to the workpiece W are removed by using air blow, ultrasonic cleaning, and the like. Through the processes, a series of drilling is terminated.

Next, description will be given of an experiment example in which drilling of the FRP was performed by using the drilling method of one embodiment. In the experiment example, processing of forming 100 pieces of holes (10 pieces × 10 pieces) which have a diameter φ of 2.0 mm (on a surface to be processed side) and have an approximately circular shape in glass fiber-reinforced glass (GFRP) workpiece W having a plate shape (200 mm × 200 mm × t1.0 mm (thickness)) was performed.

As the resist layer, a sheet (thickness: 0.5 mm), which contains an unsaturated polyurethane or an acrylic resin as a main component and in which an opening having a shape corresponding to a hole to be processed, was used.
Resist A: Unsaturated polyurethane is a main component (contained in 53 wt%)
Resist B: Unsaturated polyurethane is a main component (contained in 73 wt%)
Resist C: Acrylic resin is a main component (contained in 60 wt%)

Other main processing conditions were set as illustrated in Table 1.

**[Table 1]**

| Blasting abrasives | Silicon carbide particles (average particle size: 150 µm) |
|---|---|
| Ejecting pressure | 0.4 MPa |
| Distance between workpiece and nozzle | 100 mm |
| Angle of nozzle | 90° |
| Scanning velocity of workpiece | 100 mm/sec |
| Number of times of scanning of workpiece | 40 Pass |

After performing drilling with respect to the workpiece W, among 100 pieces of holes which were formed, arbitrary 10 pieces of holes were selected, and were observed by using an electron microscope. Then, evaluation was performed. Evaluation standards were as follows.

### <Processing Progress>

○ ··· All holes are penetrated, and an angle of a wall surface of the all holes is 80° to 90°.
△ ··· All holes are penetrated, and the angle of the wall surface of the all holes is 60° to 80°.
× ··· Hole which is not penetrated exists, or hole in which the angle of the wall surface of the hole is 59° or less exists.

### <Diameter of Hole>

○ ··· Diameter on a surface to be processed side is less than ±7% of a target dimension (φ 2.0 mm) in all holes.
△ ··· Diameter on the surface to be processed side is ±8% to ±15% of the target dimension (φ 2.0 mm) in the all holes.
× ··· Hole in which the diameter on the surface to be processed side is ±16% of the target dimension (φ 2.0 mm) exists.

### <Presence of Absence of Peeling-Off>

○ ··· All holes have a circular shape.
△ ··· Hole in which a surface-layer peeling-off trace is observed in the vicinity of an outer periphery exists, but the trace is less than 1 mm from an outer periphery of a circle.
× ··· Hole in which the surface-layer peeling-off trace is observed in the vicinity of the outer periphery exists, and the magnitude of the trace is 1 mm or greater from the outer periphery of a circle.

### <Presence or Absence of Fluffing>

○ ··· Fluffing is not confirmed in all holes.
△ ··· Hole in which slight fluffing is confirmed exists, but an exposed glass fiber is less than 0.1 mm.
× ··· Hole in which fluffing is confirmed exists, and the exposed glass fiber is 0.1 mm or greater.

Hereinafter, processing conditions and evaluation results of various examples and comparative examples are illustrated in Table 2. "Processing" in Table 2 represents an evaluation results relating to "Processing Progress", "Peeling-Off" represents an evaluation result relating to "Presence or Absence of Peeling-Off", and "Fluffing" represents an evaluation result relating to "Presence or Absence of Fluffing". In addition, "Nozzle angle" in Table 2 represents the angle of the ejection flow of the blasting abrasives with respect to the surface of the workpiece W, and 0° is an angle at which the ejection flow is horizontally ejected toward a scanning direction side in the longitudinal direction of the workpiece W at initiation of scanning. That is, a state in which the ejection flow flows in the +X direction illustrated in FIG. 3 is set as 0°.

**[Table 2]**

| | Resist Layer | d2/dl | Nozzle angle (deg.) | Evaluation | | | |
|---|---|---|---|---|---|---|---|
| | | | | Processing | Diameter of hole | Peeling-Off | Fluffing |
| Example 1 | A | 0.85 | 92 | ○ | ○ | ○ | ○ |
| Example 2 | A | 0.90 | 92 | ○ | ○ | ○ | ○ |
| Example 3 | A | 0.94 | 92 | ○ | ○ | ○ | ○ |
| Example 4 | A | 0.92 | 85 | ○ | ○ | ○ | ○ |
| Example 5 | A | 0.92 | 94 | ○ | ○ | ○ | ○ |
| Example 6 | B | 0.85 | 92 | ○ | ○ | ○ | ○ |
| Comparative Example 1 | A | 0.78 | 92 | × | ○ | ○ | ○ |
| Comparative Example 2 | A | 0.98 | 92 | ○ | △ | △ | △ |
| Comparative Example 3 | A | 1.05 | 92 | ○ | × | × | × |
| Comparative Example 4 | A | 0.92 | 79 | △ | ○ | ○ | △ |
| Comparative Example 5 | A | 0.92 | 120 | × | ○ | ○ | △ |
| Comparative Example 6 | C | 0.85 | 92 | △ | △ | △ | △ |

### (1) Influence of d₂/d₁

In Examples 1 to 6, all evaluation items were "O" evaluation, and it was confirmed that drilling was performed in a satisfactory manner. Furthermore, in a qualitative evaluation, although the evaluation was the same "O" evaluation, but Example 2 and Example 3 shown a tendency in which a diameter of a hole after processing was closer to a desired dimension in comparison to Example 1.

In Comparative Example 1 in which d₂/d₁ was smaller than 0.84, "Processing Progress" was "×" evaluation. This is assumed to be because a chance for the blasting abrasives to come into contact with the workpiece W was excessively small. In Comparative Example 2 in which d₂/d₁ was greater than 0.94, all evaluations of "Diameter of hole", "Presence or Absence of Peeling-OFF of Surface Layer", and "Presence or Absence of Fluffing" were "△" evaluation. With regard to the "△" evaluation, it can be said that quality deterioration has no problem in practical use, but the quality further deteriorates in comparison to Examples 1 to 5. In addition, in Comparative Example 3 in which d₂/d₁ was greater than 1 (that is, d₂ > d₁), evaluations of "Diameter of hole", "Presence or Absence of Peeling-OFF of Surface Layer", and "Presence or Absence of Fluffing" were "×" evaluation. It is assumed that when d₂/d₁ increases, an effect of suppressing of a processing area due to the opening of the resist layer is reduced, and thus a surface layer of the workpiece W was peeled off.

### (2) Influence of Nozzle Angle

In Examples 1 to 6, all were "O" evaluation, and it was confirmed that drilling was performed in a satisfactory manner. In Comparative Example 4 and Comparative Example 5 in which the angle exceeded 90° ± 5°, it could be seen that quality deteriorates in evaluations of "Processing Progress" and "Presence or Absence of Fluffing". With regard to "Processing Progress", it is assumed that an inclination angle of the ejection flow with respect to the workpiece W was great and processing capability deteriorated, and thus quality deteriorated. With regard to the "△" evaluation, it can be said that quality deterioration has no problem in practical use. However, in Comparative Example 5 in which the nozzle angle was relatively large, evaluation was "×". In addition, with regard to "Presence or Absence of Fluffing", it is assumed that the ejection flow flowed along the surface of the workpiece W, and thus fluffing occurred.

### (3) Influence of Material of Resist Layer

In Example 1, Example 6, and Comparative Example 6, the same processing conditions were set except for a material of the resist layer. In Example 1 and Example 6 in which a main component of the resist layer was unsaturated polyurethane, all evaluation items were "○" evaluation, and it was confirmed that drilling was performed in a satisfactory manner. Furthermore, in a qualitative evaluation, although the evaluation was the same "O" evaluation. However, there was a tendency in which the diameter of the hole after processing was closer to a desired dimension in Example 1 in which a content rate of unsaturated polyethylene was in a range of 50% to 70% in comparison to Example 6.

On the other hand, in Comparative Example 6 in which the main component of the resist layer was an acrylic resin, evaluation items of "diameter of hole", "Peeling-off", and "Fluffing" were "△" evaluation. With regard to the "△" evaluation, it can be said that quality deterioration has no problem in practical use. However, it was confirmed that processing accuracy was further lowered in comparison to a case of using a resist layer in which unsaturated polyurethane is a main component.

Hereinbefore, description has been given of the embodiments, but various modifications can be employed without limitation to the embodiments. For example, in the drilling method according to the embodiment, in the step S1, the sheet 70 in which an opening is formed in advance is disposed on the workpiece W. However, in one embodiment, the opening 71 may be formed in the sheet 70 after disposing the sheet 70, in which the opening 71 is not formed, on the workpiece W.

### Industrial Applicability

In the embodiments, description has been given of drilling with respect to the workpiece W that is constituted by glass fiber-reinforced plastic (GFRP), but the drilling method according to the embodiments is applicable to drilling of a workpiece W that is constituted by all kinds of fiber-reinforced plastics such as carbon fiber-reinforced plastic (CFRP), aramid fiber-reinforced plastic (AFRP), dyneema fiber-reinforced plastic (DFRP), xyron fiber-reinforced plastic, and boron fiber-reinforced plastic (BFRP).

### Reference Signs List

01: sandblast machine, 10: housing, 11: door, 12: nozzle fixture, 13: processing table, 14: movement mechanism, 15: frame, 20: fixed-quantity supply mechanism, 30: separation mechanism, 40: suction mechanism, 50: nozzle, 51: nozzle holder, 52: air nozzle, 53: ejecting nozzle, 60: control device, 70: sheet, 71: opening, 72: peripheral edge portion, A: ejecting region, H1: air hose, H2: blasting abrasives hose, R: processing chamber, T: scanning trajectory, W: workpiece.

## Claims

1. A drilling method of forming a hole (H) having a desired diameter (d₁) in a fiber-reinforced plastic workpiece (W), comprising steps of:
disposing a resist layer (70), in which an opening (71) having a diameter (d₂) smaller than the desired diameter (d₁) is formed, on the workpiece (W), wherein a ratio of the diameter (d₂) of the opening (71) to the desired diameter (d₁) is 0.84 or more and 0.94 or less; and
ejecting blasting abrasives to the workpiece (W) through the resist layer (70) to cut a portion, which is exposed from the opening (71), in the workpiece (W) while cutting a peripheral edge portion (72) of the opening (71) of the resist layer (70).

2. The drilling method according to claim 1,
wherein in the step of ejecting the blasting abrasives to the workpiece (W), the blasting abrasives are ejected toward the workpiece (W) from a nozzle (50), and
an angle formed by a surface of the workpiece (W) and an ejecting direction of the blasting abrasives from the nozzle is 90° ± 5°.

3. The drilling method according to claim 2,
wherein the nozzle (50) is configured to suck the blasting abrasives by introducing compressed air to the inside of the nozzle (50) to eject the blasting abrasives with the compressed air as a solid-gas two-phase flow.

4. The drilling method according to any one of claims 1 to 3,
wherein the workpiece (W) comprises the fiber-reinforced plastic in which cut reinforcing fibers are dispersed in a resin.

5. The drilling method according to any one of claims 1 to 3,
wherein the workpiece (W) comprises the fiber-reinforced plastic in which woven reinforcing fibers infiltrate into a resin.

6. The drilling method according to any one of claims 1 to 5,
wherein the resist layer (70) is a polymer including unsaturated polyurethane or an abrasion-resistant rubber as a main component.

7. The drilling method according to any one of claims 1 to 5,
wherein the fiber-reinforced plastic has a plate shape having a thickness of 1.0 mm or more and 2.0 mm or less, and
an angle formed by a plane perpendicular to a central axis line (AX) of the hole (H) and a wall surface defining the hole (H) is 80° or more and 90° or less.

## Patentansprüche

1. Bohrverfahren zum Bilden eines Loches (H), das einen gewünschten Durchmesser (d₁) aufweist, in einem faserverstärkten Kunststoffwerkstück (W), die folgenden Schritte umfassend:
Anordnen einer Resistschicht (70), in der eine Öffnung (71), die einen Durchmesser (d₂) aufweist, der kleiner als der gewünschte Durchmesser (d₁) ist, gebildet wird, auf dem Werkstück (w), wobei ein Verhältnis des Durchmessers (d₂) der Öffnung (71) zum gewünschten Durchmesser (d₁) 0,84 oder mehr, und 0,94 oder weniger beträgt; und
Ausstoßen von Strahlmitteln auf das Werkstück (W), durch die Resistschicht (70) hindurch, zum Ausschneiden eines Abschnitts, der von der Öffnung (71) freigelegt ist, in dem Werkstück (W) während des Schneidens eines umlaufenden Kantenabschnitts (72) der Öffnung (71) der Resistschicht (70).

2. Bohrverfahren nach Anspruch 1,
wobei beim Schritt des Ausstoßens von Strahlmitteln auf das Werkstück (W) Strahlmittel von einer Düse (50) zum Werkstück (W) hin ausgestoßen werden, und
ein Winkel, der durch eine Oberfläche des Werkstücks (W) und eine Ausstoßrichtung der Strahlmittel aus der Düse gebildet wird, 90° ± 5° beträgt.

3. Bohrverfahren nach Anspruch 2,
wobei die Düse (50) konfiguriert ist, um die Strahlmittel durch Einbringen von Druckluft ins Innere der Düse (50) anzusaugen, um die Strahlmittel mit der Druckluft als Feststoff-Gas Zweiphasenstrom auszustoßen.

4. Bohrverfahren nach einem der Ansprüche 1 bis 3,
wobei das Werkstück (W) einen faserverstärkten Kunststoff umfasst, in dem geschnittene Verstärkungsfasern in einem Harz verteilt sind.

5. Bohrverfahren nach einem der Ansprüche 1 bis 3,
wobei das Werkstück (W) einen faserverstärkten Kunststoff umfasst, in dem verwebte Verstärkungsfasern in ein Harz einsickern.

6. Bohrverfahren nach einem der Ansprüche 1 bis 5,
wobei die Resistschicht (70) ein Polymer ist, das ungesättigtes Polyurethan oder einen abriebfesten Gummi als Hauptkomponente umfasst.

7. Bohrverfahren nach einem der Ansprüche 1 bis 5,
wobei der faserverstärkte Kunststoff eine Plattenform aufweist, die eine Dicke von 1,0 mm oder mehr und 2,0 mm oder weniger aufweist, und
ein Winkel, der durch eine zu einer Mittelachslinie (AX) des Loches (H) senkrechte Ebene und eine das Loch (H) definierende Wandoberfläche gebildet wird, 80° oder mehr und 90° oder weniger beträgt.

## Revendications

1. Procédé de forage pour la formation d'un trou (H) ayant un diamètre souhaité (d₁) dans une pièce à travailler en matière plastique renforcée de fibres (W), comprenant les étapes consistant à :
disposer une couche de réserve (70), dans laquelle une ouverture (71) ayant un diamètre (d₂) inférieur au diamètre souhaité (d₁) est formée, sur la pièce à travailler (w), dans lequel un rapport du diamètre (d₂) de l'ouverture (71) au diamètre souhaité (d₁) s'élève à 0,84 ou plus et à 0,94 ou moins ; et
éjecter des abrasifs de décapage sur la pièce à travailler (W) à travers la couche de réserve (70) pour couper une portion qui est exposée depuis l'ouverture (71), dans la pièce à travailler (W) tout en coupant une portion de bord périphérique (72) de l'ouverture (71) de la couche de réserve (70).

2. Procédé de forage selon la revendication 1,
dans lequel dans l'étape d'éjection des abrasifs de décapage sur la pièce à travailler (W), les abrasifs de décapage sont éjectés vers la pièce à travailler (W) depuis une buse (50), et
un angle formé par une surface de la pièce à travailler (W) et une direction d'éjection des abrasifs de décapage depuis la buse s'élève à 90° ± 5°.

3. Procédé de forage selon la revendication 2,
dans lequel la buse (50) est configurée pour aspirer les abrasifs de décapage par l'introduction d'air comprimé à l'intérieur de la buse (50) pour éjecter les abrasifs de décapage avec l'air comprimé comme un flux à deux phases gaz-solide.

4. Procédé de forage selon l'une quelconque des revendications 1 à 3,
dans lequel la pièce à travailler (W) comprend la matière plastique renforcée de fibres, dans laquelle des fibres de renforcement coupées sont dispersées dans une résine.

5. Procédé de forage selon l'une quelconque des revendications 1 à 3,
dans lequel la pièce à travailler (W) comprend la matière plastique renforcée de fibres, dans laquelle des fibres de renforcement tissées s'infiltrent dans une résine.

6. Procédé de forage selon l'une quelconque des revendications 1 à 5,
dans lequel la couche de réserve (70) est un polymère incluant du polyuréthane insaturé ou un caoutchouc résistant à l'abrasion comme un composant principal.

7. Procédé de forage selon l'une quelconque des revendications 1 à 5,
dans lequel la matière plastique renforcée de fibres présente une forme plate ayant une épaisseur de 1,0 mm ou plus et de 2,0 mm ou moins, et
un angle formé par un plan perpendiculaire à une ligne d'axe central (AX) du trou (H) et une surface de paroi définissant le trou (H) s'élève à 80° ou plus et à 90° ou moins.
